



US005661880A

## United States Patent [19]

Schippers et al.

[11] Patent Number: 5,661,880

[45] Date of Patent: Sep. 2, 1997

## [54] METHOD AND APPARATUS FOR PRODUCING A MULTIFILAMENT YARN BY A SPIN-DRAW PROCESS

[75] Inventors: **Heinz Schippers; Erich Lenk**, both of Remscheid, Germany[73] Assignee: **Barmag AG**, Remscheid, Germany

[21] Appl. No.: 598,839

[22] Filed: Feb. 9, 1996

## [30] Foreign Application Priority Data

Feb. 10, 1995 [DE] Germany 195 04 422.3

[51] Int. Cl.<sup>6</sup> D01D 4/02; D01D 5/08; D01D 10/02

[52] U.S. Cl. 28/240; 28/245; 264/290.5; 264/210.8; 425/66

[58] Field of Search 28/240, 241, 243, 28/245; 264/290.5, 288.8, 210.8, 291; 425/66

## [56] References Cited

## U.S. PATENT DOCUMENTS

- 3,771,307 11/1973 Petille .  
 3,772,872 11/1973 Piazza et al. .  
 4,185,064 1/1980 Schippers 264/210.2

|           |         |                   |           |
|-----------|---------|-------------------|-----------|
| 4,235,000 | 11/1980 | Nikkel .....      | 28/241    |
| 4,731,217 | 3/1988  | Gerhardt et al. . |           |
| 4,774,042 | 9/1988  | Schippers .....   | 264/210.8 |
| 4,863,664 | 9/1989  | Burton .....      | 264/210.8 |
| 5,408,730 | 4/1995  | Yamamoto .....    | 28/240    |

## FOREIGN PATENT DOCUMENTS

|           |         |                      |
|-----------|---------|----------------------|
| 0 089 912 | 9/1983  | European Pat. Off. . |
| 19 05 507 | 8/1970  | Germany .            |
| 22 54 998 | 7/1975  | Germany .            |
| 22 41 718 | 12/1976 | Germany .            |
| 35 28 306 | 2/1986  | Germany .            |
| 1 262 813 | 2/1972  | United Kingdom .     |

Primary Examiner—Andy Falik  
 Attorney, Agent, or Firm—Bell, Seltzer, Park & Gibson,  
 P.A.

## [57] ABSTRACT

A method and apparatus for producing a multifilament yarn by a melt spinning-draw process, and which includes applying additional heat to the melt in the region of the spinneret. The relationship between the withdrawal speed and draw ratio may be changed, and with an adaptation of other process parameters, it is possible to increase productivity. The process may be applied to continuous and discontinuous processes.

16 Claims, 5 Drawing Sheets





FIG. 1.



FIG. 3.







ELONGATION AT BREAK [%] AS A FUNCTION OF  
THE WITHDRAWAL SPEED ( $\frac{1\text{Br}-1}{100}$ )  
YARN DENIER (DENIER PER FILAMENT)

|      | 0.3   | 0.5   | 1     | 2     | 4     |
|------|-------|-------|-------|-------|-------|
| 2000 | 132 % | 155 % |       |       |       |
| 2500 | 103 % | 122 % | 142 % | 153 % |       |
| 3000 | 81 %  | 96 %  | 114 % | 121 % | 138 % |
| 3500 | 70 %  | 78 %  | 91 %  | 97 %  | 110 % |
| 4000 | 63 %  | 69 %  | 76 %  | 80 %  | 90 %  |
| 4500 | 56 %  | 61 %  | 67 %  | 70 %  | 76 %  |
| 5000 | 50 %  | 54 %  | 60 %  | 63 %  | 67 %  |
| 5500 | 45 %  | 48 %  | 52 %  | 56 %  | 59 %  |
| 6000 | 40 %  | 43 %  | 48 %  | 49 %  | 52 %  |

TABLE I.



FIG. 6.

**METHOD AND APPARATUS FOR  
PRODUCING A MULTIFILAMENT YARN BY  
A SPIN-DRAW PROCESS**

**BACKGROUND OF THE INVENTION**

The present invention relates to a method and apparatus for producing a multifilament yarn from a heated thermoplastic melt.

DE-B 22 41 718 (Du Pont) and U.S. Pat. Nos. 3,771,307 and 3,772,872 disclose a method and apparatus of the described type which is characterized by the steps of melt spinning a yarn at a high withdrawal speed and then drawing the yarn, the drawing occurring along with a false twist texturing treatment.

It has been found that there exists a physical dependence between the withdrawal speed and the draw ratio that can still be realized thereafter. This interdependence occurs as a result of a partial orientation of the molecule chains that is realized by the high withdrawal speed which is in this instance more than 2,000 meters per minute. As a consequence, the elongation at break of the thus partially oriented yarn (POY) and, thus, likewise its subsequent stretchability are reduced. For a polyester yarn (polyethylene terephthalate, and others), and for a polyamide yarn (nylon 6 and nylon 6.6), the physical dependence may be noted essentially from the diagram of German Patent 22 54 998. "Normal withdrawal speed" and/or "normal draw ratio", as used hereafter, are meant to be a draw ratio, which maintains the relationships in accordance with this diagram, i.e., the partially oriented yarn is spun in conventional manner and not in accordance with the teaching of this invention.

Together with the total denier of the yarn that is to be produced, this physical dependence causes a limitation of productivity. The productivity again can be measured by the delivery or flow rate of the melt, i.e., the weight of the melt per unit time, expressed for example as grams per minute.

In a continuous spin-draw and takeup process, the increase in the withdrawal speed does not result in a corresponding increase in productivity, since as the withdrawal speed increases, the stretchability or draw ratio decreases and, consequently, the takeup speed changes only little or not at all.

In such a continuous spin-draw and takeup process, the yarn advances immediately after spinning to a draw zone, and is wound after passing through the draw zone.

In a discontinuous production process, a takeup occurs after spinning. The produced package is then supplied to a draw machine, and wound again after passing through the draw zone. In this process, the rate of flow, at which the melt is discharged, results from the total denier that must be reached at a given withdrawal speed and draw ratio. Due to the physical relationships, the conventional production process does not permit a significant increase in productivity to be realized for a yarn by melt spinning a partially oriented yarn and its subsequent drawing (see, treatise "Spinnstrecken-Schnellspinnen-Strecktexturieren" in International Textile Bulletin ITB, 1973, p. 373).

It is accordingly an object of the present invention to provide a method and apparatus for the production of a multifilament yarn which permits the production rate to be increased.

**SUMMARY OF THE INVENTION**

The above and other objects and advantages of the present invention are achieved by the provision of a method and

apparatus which includes the steps of extruding the heated melt through a spinneret at a predetermined weight flow rate so as to produce a plurality of advancing filaments, and including applying additional heat to the melt in the spinneret and/or immediately upon its exit from the spinneret.

The advancing filaments are then gathered to form an advancing yarn, and the advancing yarn is withdrawn from the spinneret at a speed of at least about 2000 m/min so as to at least partially orient the molecules of the yarn.

10 Thereafter, the advancing yarn is drawn between two feed rolls so as to impart a predetermined draw ratio, and finally, the advancing yarn is wound into a yarn package.

As important features of the present invention, the withdrawing step and the drawing step include adapting the withdrawal speed and/or the draw ratio to the changed physical relationship between the withdrawal speed and draw ratio resulting from the amount of heat applied in the step of applying additional heat to the melt. Also, the extruding step includes adapting the weight flow rate of the melt to the adapted withdrawal speed and/or the adapted draw ratio such that a predetermined total denier is attained.

15 In one embodiment, the process is a continuous production process. In such a case, the desired total denier of the yarn to be produced and the desired flow rate of the melt result in the takeup speed of the yarn, which corresponds substantially to the final speed in the draw zone. By inputting a desired draw ratio, the withdrawal speed of the yarn from the spinneret is obtained, or vice versa, by inputting a desired withdrawal speed, the draw ratio is obtained in both cases in accordance with the predetermined physical relationship. Only the measure as provided by the present invention results in an increase in productivity to a noteworthy extent, since it allows to break the described physical relationship between withdrawal speed and draw ratio.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 98

in the spinning phase without raising the takeup speed, but with an increased denier of the partially oriented yarn, and the yarn being drawn in the drawing phase at an increased draw ratio. Thus, in the drawing phase, the produced yarn length is likewise increased, while the total denier remains unchanged. In the other alternative, the increase in the flow rate of the melt results in an increase of the takeup speed and, thus, in an increase in productivity, in the spinning phase. The subsequent drawing occurs in the usual manner.

An important feature of the invention is the fact that the molten state of the melt strands emerging from the nozzle holes of the spinneret and becoming subsequently individual filaments is still maintained over a length, even though the length is short. It is possible that this may similarly occur where relatively large diameters are used for the nozzle holes in the spinneret. In accordance with the invention, however, the increase in productivity may be achieved in operationally reliable manner only by a supply of heat.

The heat may be supplied to the melt upon its exit from the spinneret by directing a current of heated air or gas against the melt strands, with the current being directed perpendicularly to the melt strands or transversely thereto with a component directed toward the underside of the spinneret. This embodiment has the advantage that the actual spinning apparatus need not be modified, and that the heating zone may be extended to any desired length and according to requirements.

However, in this process undesirable evaporation of monomers and oligomers may develop, which deposit on the underside of the spinneret and adversely affect the reliability of the process.

To avoid this disadvantage, the heat may be supplied by heating the spinneret, to an extent to at least compensate for the heat loss of the spinneret normally incurred as the result of the usual cooling air flow, radiation, etc. This procedure prevents primarily the molecules from becoming oriented in the spinneret. In this connection, it should be noted that the partial orientation of the yarn or the yarn molecules is also caused largely by the flow conditions in the narrow nozzle holes of the spinneret. The heating of the spinneret prevents this flow orientation from solidifying and leading to a corresponding partial orientation.

It is believed that the spinneret should be heated by more than 5° C., preferably 5° to 30° C. In the tests, heating was at about 10° C.

DE-OS 19 05 507 teaches that a spinneret may be heated for compensating for the heat losses in a conventional spinning process at low withdrawal speeds and without partial orientation of the yarn. In the present invention, the spinneret may be heated, for example, by providing resistance heating wires in or on the spinneret. The resistance heating wires may then be operated at a desired temperature.

The heat may also be supplied to the spinneret by infrared radiation, by positioning an annular metallic member below the spinneret, and heating the member to a temperature sufficient to emit infrared radiation. This has the advantage that the spinning apparatus need not be modified to a significant extent. Moreover, it prevents contaminations, oligomers, and monomers from depositing on the spinneret, and it ensures that the spinneret is evenly heated over its entire surface.

The radiation heater may be mounted by a hinge so as to permit it to be selectively opened and thereby provide access to the spinneret for cleaning and for removing deposits by scraping.

#### BRIEF DESCRIPTION OF THE DRAWINGS

Some of the objects and advantages of the present invention having been stated, others will appear as the description

proceeds, when considered in conjunction with the accompanying drawings, in which:

FIG. 1 is a schematic view of a continuous spin and draw process for producing a flat yarn;

FIGS. 2 and 3 are schematic views of a two-step process for spinning a partially oriented, flat yarn and for subsequently draw texturing the partially oriented yarn in a second process step;

FIG. 4 is a sectional view of the region of the spinneret;

FIG. 5 is a diagram illustrating, in accordance with Table 1, the relationship between withdrawal speed and elongation at break for partially oriented polyester yarns with different filament deniers; and

FIG. 6 is a diagram illustrating the dependence of the increase in elongation at break on the total denier of the produced yarn with a predetermined supply of heat to the spinneret.

#### DETAILED DESCRIPTION OF THE PREFERRED EMBODIMENTS

The processes described below are equally suitable for spinning yarns of polyester or polyamide. A polyester may be in particular polyethylene terephthalate. Used as polyamides are in particular nylon 6 (Perlon<sup>TM</sup>) and nylon 6.6. It should be expressly remarked that the process data indicated below are for polyester. They apply accordingly to polyamide yarns with deviations that are to be established by tests.

Described below is the spinning process. This description of the spinning process applies to both the embodiment of FIG. 1 and the embodiment of FIG. 2, except deviations as will be expressly identified.

A yarn 1 is spun from a thermoplastic material. The thermoplastic material is supplied through a hopper 2 to an extruder 3. The extruder 3 is driven by a motor 4, which is controlled by a control unit 8. In the extruder, the thermoplastic material is melted. The work of deformation, which is applied by the extruder, assists in the melting process on the one hand. In addition, a heater 5 in the form of a resistance heater is provided, which is controlled by a heating control unit 43. Through a melt line, the melt reaches a gear pump 9, which is controlled by a pump motor 44. The melt pressure before the pump is detected by a pressure sensor 7, and maintained constant by feeding the pressure signal back to motor control unit 8.

The pump motor is controlled by a control unit 45 such as to permit a very fine adjustment of the pump speed. The pump 9 transports the melt flow to a heated spin box 10, the underside of which mounts a spinneret 11 accommodated in a spin pack 53 (note FIG. 4). From spinneret 11, the melt emerges in the form of fine filament strands 12. The filament strands advance through a cooling shaft 14. In the cooling shaft 14, an air current 15 is directed transversely or radially to the web of filaments, thereby cooling the filaments.

At the outlet of cooling shaft 14, the web of filaments is combined by an applicator roll 13 to a yarn 1, thereby receiving a liquid spin finish. The yarn is withdrawn from cooling shaft 14 and from spinneret 11 by a godet 16. The yarn loops several times about the godet. To this end, a guide roll 17 is used, which is axially inclined relative to godet 16. The guide roll 17 is freely rotatable. The godet 16 is driven at a preadjustable speed by a motor 18 and a frequency changer 22. This withdrawal speed is by a multiple higher than the natural exit speed of the filaments from spinneret 11.

The adjustment of the input frequency of frequency changer 22 allows to adjust the rotational speed of godet 16, thereby determining the withdrawal speed of yarn 1 from spinneret 11.

Up to this point, the description applies in like manner to the spinning process shown in FIG. 2. For the drawing step in the schematic illustration of FIG. 1, the following description applies:

Downstream of godet 16 is a draw roll or godet 19 with a further guide roll 20. With respect to their arrangement, both correspond to that of godet 16 with guide roll 17. Draw roll 19 is driven by a motor 21 with a frequency changer 23. The input frequency of frequency changers 22 and 23 is evenly preset by a controllable frequency changer 24. In this manner, it is possible to individually adjust on frequency changers 22 and 23 the speed of godet 16 and draw roll 19 respectively, whereas the speed level of godet 16 and draw roll 19 is adjusted collectively on frequency changer 24.

From draw roll 19, the yarn 1 advances to a so-called "apex yarn guide" 25, and thence into a traversing triangle 26.

The following description will apply in like manner to the takeup step in the process of FIG. 1 and in the process of FIG. 2. In both Figures, the yarn traversing mechanism is not shown.

The traversing mechanism may be, for example, a cross-spiralled roll with a yarn guide traversing therein and reciprocating the yarn over the length of a package 33. In so doing, the yarn loops about a contact roll 28 downstream of yarn traversing mechanism 27. The contact roll 28 rests against the surface of package 33. It is used to measure the surface speed of package 33. The package 33 is wound on a tube 35, which is clamped on a winding spindle 34. The spindle 34 is driven by a motor 36 and a spindle control unit 37 such that the surface speed of package 33 remains constant. To this end and for use as a control variable, the speed of freely rotatable contact roll 28 is sensed and corrected by means of a ferromagnetic insert 30 and a magnetic pulse transmitter 31.

In the process of FIG. 1, the adjustment of spindle control unit 37 allows to adapt the takeup speed to the circumferential speed of draw roll 19.

In the embodiment of FIG. 2, the yarn advancing from godet 16 moves on directly to apex yarn guide 25 and into the traversing triangle 26. In this embodiment, an adaptation occurs in corresponding manner between the circumferential speed of package 33 and the withdrawal speed, which is predetermined by godet 16.

In both cases, the circumferential speed of package 33, which is sensed and corrected by contact roll 28, is slightly lower than the circumferential speed of preceding godets 16 or 19, since the takeup speed of the yarn results as a geometric sum from the circumferential speed of package 33 and the traversing speed of yarn traversing mechanism 27 which is not shown.

FIG. 3 is a schematic illustration of a draw-texturing process. The package 33 with a partially oriented yarn, which was produced by the spin process of FIG. 2, is supplied to a draw-texturing machine. Yarn guides 38 advance the partially oriented yarn to a first feed system 39, from where the yarn passes through a heater 46, a cooling rail 47, a friction false twist unit 48, to a second feed system 50, so as to be subsequently wound to a package 52. The feed systems 39 and 50 are driven at different speeds. As a result, the necessary drawing occurs in the false twist zone between these feed systems along with a heating and a false twist texturing.

In the following, the processes of FIGS. 1 and 2 or 3 are described in more detail.

Referring now to FIG. 1, a continuous spin-draw process is shown. In this process, the total denier results from the takeup speed and the flow rate of the melt.

For example, a yarn having a total denier of 2 denier per filament is to be produced. The withdrawal speed is to be 3000 m/min. Under normal circumstances, i.e. without heating the spinneret, this results in an elongation at break of the produced yarn of 120%. In other words, this means that the withdrawn, partially oriented yarn can be drawn to 220% of its length before breaking. As a consequence thereof, the draw ratio is about two thirds of this value, namely, for example 1:1.6.

10 This results in a withdrawal speed of 4800 m/min. (3000 m/min $\times$ 1.6=4800 m/min). With a filament having, as aforesaid, a weight per unit length measure of 2 denier per filament and a number of 72 filaments, the result is a total denier of 150. From this, the flow rate of the melt for each spinning position is 150 g/9000 m $\times$ 4800 m/min=80 g/min. Assuming now that the withdrawal speed for the production of the same yarn is increased to 4000 m/min, the elongation at break will be 80%, i.e., the yarn can be drawn to 180% of its length before breaking. When a draw ratio having again 15 an approximate range of two thirds is selected, the draw ratio will be 1:1.2. This means that the withdrawal speed is not increased.

15 It is obvious that the flow rate of the melt discharged from the pump cannot be increased in the production of the same total denier. Therefore, the increase in production or productivity is irrelevant.

20 For this reason, a radiation heater is used below the spinneret, as shown in FIG. 4. In the following this radiation heater is described in like manner for the process of FIGS. 1 and 2. The spinneret 11 is located in a nozzle pack 53. The nozzle pack 53 is accommodated in spin box 10, which is heated. Details are not shown. Arranged below the spinneret and directly adjacent thereto is a radiation heater 56, which is constructed as a ring and made of steel. Its inside surface 30 58 directed toward the center is formed by a conical surface, which faces the spinneret. A suitable angle of cone (total angle) is, for example, from 30° to 40°. Inserted into the radiation heater is an annular heating strip 57, which may be a resistance heating wire. This resistance heating wire permits to heat the radiation heater to redness at temperatures from above 300° to about 800° C. Very effective temperatures are in a range from 450° to 700° C.

25 Subjacent the radiation heater is air cooling 51 as has been described above.

30 It shows now that at the same withdrawal speed of 3000 m/min and with a radiation toward the spinneret by means of the heated element, a substantial increase in the elongation at break will occur and, as a result, likewise an increase in the draw ratio of the yarn. With a radiation from the heater heated to 550° C., it was possible to increase in the example the elongation at break and, thus, the draw ratio by 5%. Thus, a withdrawal speed of 3000 m/min resulted in a takeup speed likewise increased by 5%, namely of 3040 m/min. In 35 the production of the initially indicated yarn denier, this increased takeup speed requires an increase of the melt delivery by discharge pump 9 to 84 g/min. As a result, the productivity of the system can be increased by 5%, by the simple measure of radiating heat toward the spinneret.

40 As shown in the diagram of FIG. 6, the extent of the increased productivity is dependent, on the one hand, on the radiation temperature, and on the other hand on the yarn denier. At higher yarn deniers, the effect is less, or it will be necessary to select a higher radiation temperature. In the individual case, the correlation is to be determined by test.

45 The procedure in the method shown in FIG. 2 is as follows:

For example, a 55 f 109 textured yarn, namely a yarn having 55 denier and 109 individual filaments is to be produced. This means that each yarn has 0.5 denier per filament (DPF). A draw ratio of 1.6 is determined to be optimal for the draw texturing process. This draw ratio permits a good crimping and a reliable texturing process without filament breakages. This draw ratio means that a partially oriented yarn having a denier of 88 and 109 filaments is to be supplied from feed yarn package 33. To partially orient such a yarn, so as to be able to maintain the draw ratio of 1.6, it will be necessary to adjust a  $\frac{1}{2}$  to  $\frac{1}{3}$  higher elongation at break. At a draw ratio of 1.6, the elongation at break must be 120%. From the diagram of FIG. 5 or the Table, the corresponding withdrawal speed is 2600 m/min, which must be adjusted in a method according to FIG. 2 at draw rolls 16. To produce an 88-denier, partially oriented yarn at 2600 m/min, it is necessary to adjust the flow rate of the melt on the pump to 25.5 g/min for each spinning position. An increase in the flow rate of the melt is not possible, since it will change likewise the withdrawal speed and, thus, the draw ratio. Thus, the draw ratio that is predetermined by the texturer or throwster, limits the productivity of the producer of the partially oriented yarn.

However, it is a different matter, when a radiation heater as shown in FIG. 4 is used. At the same draw ratio, it is possible to achieve an increase in the withdrawal speed by 20%, namely to 3360 m/min, in that heat is radiated toward the spinneret by the heater of FIG. 4 at a temperature of approximately 550° C. The flow rate of the melt is to be increased accordingly to 32.9 m/min. As a result, productivity is increased by more than 20% with an otherwise unchanged machine layout.

Alternatively, a textured yarn of 55 denier and 109 filaments is to be produced, however, without exceeding in the takeup zone the withdrawal speed and the takeup speed of 3000 m/min. The reason for such limitations lies in occasional process problems with sensitive yarns. Such problems may however be caused by the mechanical layout of the takeup machine, whose maximum speed is limited.

As can be noted from Table 1 or the diagram of FIG. 5, this yarn has an elongation at break of 96%. Therefore, the draw ratio to be selected in the draw zone is about two thirds of the breaking length of 196%. Selected is a draw ratio of 1.3:1. It results therefrom that the denier of the partially oriented yarn, that is supplied as feed yarn in the draw texturing process, must amount to  $55 \text{ dtex} \times 1.3 = 71.5$  denier. From this, it results again that this yarn is produced in the spin zone at a flow rate of the melt amounting to  $71.5 \text{ g} / 9000 \text{ m} \times 3000 \text{ m/min} = 23.8 \text{ g/min}$  per spinning position.

When a radiation heater of FIG. 4 is now used again, and operated at a temperature of 550° C., a 20% increased elongation at break of  $96\% \times 1.2 = 115\%$  is obtained at a withdrawal speed of 3000 m/min, namely a breaking length of 215%. Thus, in the subsequent drawing phase, it is possible to adjust the draw ratio at about two thirds of this value, i.e. to 1.45. This again means that to produce a total denier of 55 denier, it is necessary to supply as feed yarn a partially oriented yarn with a denier of  $55 \times 1.45 = 79$  denier. To produce a 79 denier yarn at a withdrawal speed of 3000 m/min, it is necessary to adjust the flow rate of the melt to 26.3 g/min per spinning position. As a result, the productivity in the spinning phase can be increased by  $26.3 - 23.8 = 2.5$  g/min per spinning position.

It should be remarked that individual values forming the basis for the preceding calculation and examples were determined for a certain polymer (polyester). As a function

of origin and the kind of polymer in use, deviations may result for the individual values, which are to be determined by test. This applies on the one hand to the determined elongations at break, the dependence of the draw ratio on the determined elongation at break, the correlation of elongation at break and denier of individual filaments, the correlation of radiation temperature and increase in the elongation at break, and likewise to the denier-related increase in productivity.

Thus, an important characteristic of the invention is the fact that the melt is heated in the spinneret. To this end, the spinneret is heated in addition to the heat, which it receives from the melt, the surrounding spin pack, and the surrounding spin box. Preferably, the temperature of the spinneret is increased by at least 5° C. and up to 40° C. In tests, increases in the temperature by 8° to 20° C. have shown to be advantageous. The basis to proceed from is always the temperature that results from the melt contacting the spinneret and the heated spin box. Normally, at a relatively low temperature of the spinneret, the heating must accordingly be greater by an additional supply of heat.

Compensated for are not only losses in heat radiation on the underside of the spinneret, but also an additional increase in temperature occurs. Whereas in a conventional process, temperatures of about 290° C. were measured on the underside of the spinneret, a radiation from a radiator heated to 550° C. resulted in an increased temperature of 310° C. The radiation heater has shown to be especially reliable in operation. However, it is also to presume that resistance heating wires may be laid in the spinneret, which permit a corresponding heating of the spinneret. The disadvantages of such a realization, in particular the problems in the manufacture are obvious. On the other hand, the spinneret is easy to clean in this instance. In comparison therewith, the annular radiation heater has the advantage that it prevents on the one hand the spinneret and in particular its underside from being directly exposed to the subjacent air cooling. On the other hand, an adequate air exchange occurs inside the annular radiation heater, so as to remove vapors, in particular monomer and oligomers, and to prevent unacceptable deposits on the underside of the spinneret. For cleaning the underside of the spinneret, the radiation heater is unilaterally arranged on a hinge, so that it can be opened downward.

That which is claimed is:

1. A method of producing a multifilament yarn from a heated thermoplastic melt comprising the steps of extruding the heated melt through a spinneret at a predetermined weight flow rate so as to produce a plurality of advancing filaments, and including applying additional heat to the melt in the spinneret and/or immediately upon its exit from the spinneret, gathering the advancing filaments to form an advancing yarn, withdrawing the advancing yarn from the spinneret at a speed of at least about 2000 m/min so as to at least partially orient the molecules of the yarn, drawing the advancing yarn between two feed rolls so as to impart a predetermined draw ratio, and winding the advancing yarn into a yarn package, wherein the withdrawing step and the drawing step include adapting the withdrawal speed and/or the draw ratio to the changed physical relationship between the withdrawal speed and draw ratio resulting from the amount of heat applied in the step of applying additional heat to the melt, and wherein the extruding step includes adapting the weight flow rate of the melt to the adapted withdrawal speed

and/or the adapted draw ratio such that a predetermined total denier is attained.

2. The method as defined in claim 1 wherein the step of applying additional heat to the melt includes heating the spinneret.

3. The method as defined in claim 2 wherein the step of heating the spinneret includes directing infrared radiation to the underside of the spinneret.

4. The method as defined in claim 3 wherein the step of directing infrared radiation to the underside of the spinneret includes positioning an annular metallic member immediately below the spinneret, with the annular metallic member including a conical radiation surface which faces the underside of the spinneret, and heating the annular metallic member.

5. The method as defined in claim 1 wherein the step of applying additional heat to the melt includes directing a stream of heated air or gas transversely across the underside of the spinneret so as to engage the melt immediately upon exiting from the spinneret.

6. The method as defined in claim 5 wherein the step of directing a stream of heated air or gas includes directing the stream so as to have a component directed toward the underside of the spinneret.

7. A method of producing a multifilament yarn from a heated thermoplastic melt comprising the steps of:

extruding the heated melt through a spinneret at a predetermined weight flow rate so as to produce a plurality of advancing filaments, and including applying additional heat to the melt in the spinneret and/or immediately upon its exit from the spinneret,

gathering the advancing filaments to form an advancing yarn,

withdrawing the advancing yarn from the spinneret at a speed of at least about 2000 m/min so as to at least partially orient the molecules of the yarn,

winding the partially oriented yarn into a package,

unwinding the partially orientated yarn from the package,

drawing the unwound partially oriented yarn by advancing the same between two feed rolls so as to impart a predetermined draw ratio, then

winding the yarn into a finished yarn package,

wherein the withdrawing step and the drawing step include adapting the withdrawal speed and/or the draw ratio to the changed physical relationship between the withdrawal speed and draw ratio resulting from the amount of heat applied in the step of applying additional heat to the melt, and

wherein the extruding step includes adapting the weight flow rate of the melt to the adapted withdrawal speed and/or the adapted draw ratio such that a predetermined total denier is attained.

8. The method as defined in claim 7 wherein the step of applying additional heat to the melt includes heating the spinneret.

9. The method as defined in claim 8 wherein the step of heating the spinneret includes directing infrared radiation to the underside of the spinneret.

10. The method as defined in claim 9 wherein the step of directing infrared radiation to the underside of the spinneret includes positioning an annular metallic member immediately below the spinneret, with the annular metallic member including a conical radiation surface which faces the underside of the spinneret, and heating the annular metallic member.

11. The method as defined in claim 7 wherein the step of applying additional heat to the melt includes directing a stream of heated air or gas transversely across the underside of the spinneret so as to engage the melt immediately upon exiting from the spinneret.

12. The method as defined in claim 11 wherein the step of directing a stream of heated air or gas includes directing the stream so as to have a component directed toward the underside of the spinneret.

13. An apparatus for producing a multifilament yarn comprising:

20 an extruder for heating and melting a thermoplastic material to form a heated melt,

an adjustable feed pump connected to the extruder for delivering the heated melt at an adjustable weight flow rate,

a spinneret connected to the output of said feed pump so as to produce a plurality of advancing filaments from the melt,

means for applying additional heat to the melt in the spinneret and/or immediately upon exiting from the spinneret,

guide means for gathering the advancing filaments to form an advancing yarn,

means for withdrawing the advancing yarn from the spinneret at a speed of at least about 2000 m/min so as to at least partially orient the molecules of the yarn,

means downstream of the withdrawing means for drawing the advancing yarn so as to impart a predetermined draw ratio to the advancing yarn, and

a winder for winding the advancing yarn into a yarn package.

14. The apparatus as defined in claim 13 wherein said means for applying additional heat to the melt comprises an annular metallic member mounted immediately below the spinneret, with the annular metallic member including a conical radiation surface which faces the underside of the spinneret, and means for heating the annular metallic member.

15. The apparatus as defined in claim 14 wherein said spinneret is mounted to a spin box, and said annular metallic member is pivotally mounted to said spin box so as to permit access to the spinneret for cleaning thereof.

16. The apparatus as defined in claim 13 wherein said means for applying additional heat to the melt comprises means for directing a stream of heated air or gag transversely across the underside of the spinneret so as to engage the melt immediately upon exiting from the spinneret.